

# UNITED STATES PATENT OFFICE.

PAUL GOLDBERG, OF BERLIN-TREPTOW, PAUL ONNERTZ, OF BERLIN-WILMERSDORF, AND ALFRED PETERS, OF BERLIN, GERMANY, ASSIGNORS TO ACTIEN GESELLSCHAFT FUR ANILIN FABRIKATION, OF BERLIN, GERMANY.

## METHOD OF PROTECTING ANIMAL FIBERS FROM THE INJURIOUS EFFECT OF ALKALINE LIQUIDS.

1,419,497.

Specification of Letters Patent. Patented June 13, 1922.

No Drawing.

Application filed August 15, 1921. Serial No. 492,492.

To all whom it may concern:

Be it known that we, PAUL GOLDBERG, PAUL ONNERTZ, and ALFRED PETERS, citizens of the German Republic, residing at Treptower Park 49, Berlin-Treptow, Germany; Dusseldorferstr. 72, Berlin-Wilmersdorf, Germany, and Grober-Ufer 4, Berlin SO. 33, Germany, have invented certain new and useful Improvements in Methods of Protecting Animal Fibers from the Injurious Effect of Alkaline Liquids (for which we have filed applications in Germany Aug. 22, 1917, and May 22, 1920), of which the following is a specification.

15 Our present invention relates to a method of protecting animal fibers from the known injurious effect which occurs when they are treated with alkaline liquids, for instance for the purposes of washing wool, degumming 20 silk, mercerizing cotton in half-wool or half-silk fabrics, fulling wool, dyeing and printing animal or mixed fibers with sulfurized dyes or vat dyes, finishing, dyeing or improving skins or leather.

25 The new method consists in adding to the alkaline liquid sulfite-cellulose waste liquor. Instead of sulfite-cellulose waste liquor the active substances contained in it may be used, such as sodium lignin-sulfonate, cell 30 pitch, sugars.

Thus in degumming silk it is possible to use caustic alkali or alkali sulfid instead of the usual solution, if by the aforesaid addition solvent action of the alkaline liquid 35 is limited to the silk-gum and destruction of the silk substance prevented. By boiling the silk for two hours with caustic soda lye of 2° Baumé specific gravity with addition of sulfite-cellulose waste liquor, a complete 40 degumming is obtained and even a further boiling for 2 hours does not affect the lustre or the other properties of the silk. By use of stronger alkali solutions the duration of treatment may be shortened even at lower 45 temperatures. Half-silk goods may be degummed in this manner and at the same time so far mercerized that the cotton fibers acquire an enhanced affinity for dyestuffs.

The process has a particular value in vat 50 dyeing. The sodium hydrosulfite vat has had only a limited field in dyeing wool because it is difficult to adjust the proportion of alkali so exactly that the dye remains

dissolved, the fiber is improved in appearance as much as possible and the dyeing 55 and fastness of the dyeings to rubbing and washing are not unfavorably affected. There have not been lacking, therefore, attempts to diminish the caustic action of the alkali of the vat on the fiber in respect of 60 the improvement of the appearance of the fiber and of the dyeing. The processes proposed, however, have not come into use. An exception is the ammonia-blue-hydrosulfite 65 vat, which, however, suffers from the objection that the preparation of the vat is troublesome and the process is limited to the use of particular vat preparations. By the present invention the alkaline hydrosulfite 70 vat is applicable, without limitation to the use of dyestuffs in particular forms and without damage of the animal fiber. Besides the protective action on the fiber, the addition of sulfite-cellulose waste liquor, for example, in indigo dyeing, produces a remarkable 75 deepening of the dyeing without detracting from the fastness thereof, so that wool can be dyed in one immersion dark blue of a good fastness to washing, fulling 80 and rubbing.

In order to illustrate in what manner the invention may be executed, without limiting it, the following examples are given:

### Example 1. Washing wool.

1 kg. of raw wool is treated during half an hour at 50° C. with a solution of 80 g. calcined sodium carbonate, 40 g. of sodium lignin-sulfonate and 40 g. of maltose in 20 90 litres of water. The wool is squeezed and rinsed until the water remains clear.

### Example 2. Degumming silk.

Raw silk is treated during 1½ hours at 95 90-95° C. with a bath containing in a litre 25 ccm. caustic soda-lye of 40° Baumé and 250 ccm. sulfite-cellulose waste liquor of 27.5° Baumé. The silk is then subsequently rinsed with water, with a diluted acid and 100 again with water.

### Example 3. Degumming silk and mercerizing cotton at the same time.

Half-silk fabrics, after being wetted, are 105 treated during 10 minutes at ordinary tem-

perature with a bath containing in a litre 590 ccm. caustic soda-lye of 40° Bé. and 250 ccm. sulfite cellulose-waste liquor of 27.5° Baumé. Then the fabrics are rinsed and 5 acidified.

*Example 4. Dyeing cotton in half-wool fabrics with sulfur dyes.*

To 900 litres of water first 900 g. calcined 10 sodium carbonate, then 3 kg. sulfur black-brown N extra conc. AGfA, dissolved with 6 kg. crystallized sodium sulfid in boiling water, 12 kg. maltose and finally 27 kg. crystallized sodium sulfate are added. In 15 this bath 30 kg. half-wool, previously well wetted are dyed during an hour at 30-40° C. Only the cotton is practically dyed deep brown.

*Example 5. Dyeing silk or half-silk with sulfur dyes.*

One proceeds as indicated in the Example 4 but dyes at a higher temperature, for instance at 50 to 80° C.

*Example 6. Dyeing of 25 kg. wool yarn with indigo.—A. Dye solution.*

2.5 kg. indigo pure BASF powder are mixed with 25 litres of water of 60° C. 30 Then 3 litres of caustic soda lye of 40° Baumé and whilst stirring 2.5 kg. of sodium hydrosulfite conc. are added. By warming at 60 to 65° C. a yellow solution occurs.

*B. Dyeing bath.*

35 3000 litres of water of 50° C. is added with 50 ccm. of caustic soda-lye of 40° Bé. and 150-200 g. of sodium hydrosulfite conc. Then dye solution, prepared as above, 40 and finally 26 kg. sulfite-cellulose waste liquor of 34° Baumé are added.

The well wetted yarn is handled in this bath during 20-30 minutes, squeezed, exposed to the air, rinsed, acidified and dried.

*Example 7. Dyeing 10 kg. loose wool with vat red B.—A. Dye solution.*

1 kg. vat red B BASF paste is mixed with 2 litres of water of 60° C. and 250 ccm. of 50 caustic soda lye of 40° Baumé. Whilst stirring 200 g. sodium hydrosulfite conc. powder are added, after a short time yellow dissolution being formed.

*B. Dyeing bath.*

55 1000 litres of water of 50° C. are added with 15 ccm. of caustic soda lye of 40° Bé. and 200 250 g. of sodium hydrosulfite

conc. Then the dye solution and finally 6.5 kg. of sulfite cellulose waste liquor of 34° 60 Baumé are added.

In this bath the wool is dyed 20-30 minutes at 50° C., then squeezed, oxidized at the air, rinsed, acidified and dried.

*Example 8. Preparing skins to be dyed.* 65

The skins are treated over night with a solution containing in a litre caustic soda-lye of 1° Baumé 100 g. maltose or 50 g. of sodium lignin-sulfonate and 50 g. maltose 70 and then washed.

*Example 9. Dyeing skins.*

The skins prepared as indicated in Example 8 are mordanted by immersing for 6 75 hours into a solution containing 2 g. potassium bichromate, 1 g. acid potassium tartrate and 0.25 g. copper sulfate in a litre of water. The well rinsed skins then are dyed in a bath containing in one litre of 80 water 2.5 g. ursol P, 0.5 g. ursol D, 2.5 ccm. ammonia of 25% strength, 60 ccm. hydrogen peroxide of 3% strength, 0.75 g. maltose and 0.75 g. sodium lignin-sulfonate.

After dyeing during 4 hours the dyed 85 skins are rinsed and finished as usual.

Having now described our invention, what we claim is,—

1. The method of protecting animal fibers from the injurious effect of alkaline liquids 90 which consists in adding sulfite cellulose waste liquor to the alkaline liquids.

2. The method of protecting animal fibers from the injurious effect of alkaline liquids 95 which consists in adding the active substances contained in sulfite cellulose waste liquor to the alkaline liquids.

3. The method of protecting animal fibers from the injurious effect of alkaline liquids 110 which consists in adding sodium lignin sulfonate and sugars contained in sulfite cellulose waste liquor to the alkaline liquids.

4. The method of protecting animal fibers from the injurious effect of alkaline liquids 115 which consists in adding sugars contained in sulfite cellulose waste liquor to the alkaline liquids.

In testimony whereof we affix our signatures in presence of two witnesses.

PAUL GOLDBERG.  
PAUL ONNERTZ.  
ALFRED PETERS.

Witnesses:

DR. ORUCERFOK,  
OTTO GALISCH.